

Aug. 16, 1949.

W. B. COOPER ET AL

2,478,964

## ANNEALING AND CLEANING COLD ROLLED STRIP STEEL

Filed Nov. 24, 1944

6 Sheets-Sheet 1

Fig. 1.



Inventors:

William B. Cooper.  
Edward J. Seibold.

By Lee human, Darby & Bushman.  
Eltonians

Attorneys

Aug. 16, 1949.

W. B. COOPER ET AL

**2,478,964**

## ANNEALING AND CLEANING COLD ROLLED STRIP STEEL

Filed Nov. 24, 1944

6 Sheets-Sheet 2



Inventors:

William B. Cooper.  
Edward J. Seabold

By Luckman Darby Luckman.  
Elmwood.

Aug. 16, 1949.

W. B. COOPER ET AL

2,478,964

ANNEALING AND CLEANING COLD ROLLED STRIP STEEL

Filed Nov. 24, 1944

6 Sheets-Sheet 3

Fig. 6.



Fig. 4.



Fig. 5.



Fig. 8.



Inventors:

William B. Cooper,  
Edward J. Seabold.

By Lushman Darby, Lushman.

Attorneys

Aug. 16, 1949.

W. B. COOPER ET AL

2,478,964

ANNEALING AND CLEANING COLD ROLLED STRIP STEEL

Filed Nov. 24, 1944

6 Sheets-Sheet 4

Fig. 10.



Fig. 9.

110



Inventors:

William B. Cooper,  
Edward J. Seabold.

Aug. 16, 1949  
Darby & Buchanan,  
Attorneys

Aug. 16, 1949.

W. B. COOPER ET AL

2,478,964

ANNEALING AND CLEANING COLD ROLLED STRIP STEEL

Filed Nov. 24, 1944

6 Sheets-Sheet 5

Fig. 11.



Fig. 12. Fig. 13.



Fig. 14.



Fig. 15.



Fig. 15.



Fig. 16.



Fig. 17.



Inventors:

William B. Cooper,  
Edward J. Seabold.

By Larkman Darby, Larkman.

Attorneys

Aug. 16, 1949.

W. B. COOPER ET AL

2,478,964

## ANNEALING AND CLEANING COLD ROLLED STRIP STEEL

Filed Nov. 24, 1944

**6 Sheets-Sheet 6**

Fig. 21.



Fig. 22.



Fig. 23.



Inventors:

William B. Cooper.  
Edward J. Seabold.

By Cochran Darby, Cochran,  
Attorneys

## UNITED STATES PATENT OFFICE

2,478,964

ANNEALING AND CLEANING COLD ROLLED  
STRIP STEEL

William B. Cooper and Edward J. Seabold, Baltimore, Md., assignors to Crown Cork & Seal Company, Inc., Baltimore, Md., a corporation of New York

Application November 24, 1944, Serial No. 565,014

9 Claims. (Cl. 263—3)

1

The present application is a continuation-in-part of our pending application Serial No. 497,524 which, in turn, is a division of our prior application Serial No. 328,292, filed April 6, 1940, now Patent No. 2,345,181, March 28, 1944. This application is directed to subject matter divisible from the former applications and to certain additional improvements as to method and apparatus, not shown or described in the prior applications, but which cooperate with the subject matter thereof.

The invention relates to methods of and apparatus for continuously handling and annealing strip steel.

More particularly, the invention is concerned with means for and methods of continuously bright-annealing low carbon, cold rolled strip steel.

It is an object of the invention to provide an improved continuous annealing method to take the place of conventional batch annealing processes, thereby to improve the quality and uniformity of the anneal, as well as to shorten the annealing time and reduce its cost.

It is a further object to increase the tonnage of strip steel that may be annealed in a given length of time with an apparatus occupying a particular area of plant space.

It is a further object of the invention to reduce greatly the cost of annealing strip steel, by materially reducing the heating costs, the handling costs and other labor charges.

It is a further object of the invention to produce in the strip steel an improved anneal, characterized by small, uniform grain structure, resulting from the use of high annealing temperatures followed by rapid cooling from the critical temperature to substantially room temperature. In accordance with the invention, the material is maintained at a high annealing temperature for a sufficient period of time to permit the crystalline grains to lose the orientation and elongated shape acquired in cold rolling, and to assume the random positions characteristic of well-annealed steel, but the steel is cooled with sufficient speed to prevent the formation of large grains of ferrite, which is a characteristic result of the long cooling periods used in batch annealing.

It is a further object of the invention to provide novel, improved means for accurately and uniformly controlling the temperature to which the strip is raised during its treatment, the time during which the strip is held or "soaked" at a high temperature, and the time, rate and degree of cooling.

2

It is a further object of the invention to provide novel means for preventing or controlling oxidation of the strip during the annealing process, whereby a bright-annealed strip or a strip having desired, controlled color characteristics, may be produced.

One of the principal objects and advantages of the present invention is the elimination, in a continuous annealing method, of fluctuations in the temperature to which the strip is subjected, whereby inequalities in the ductility and hardness of the annealed strip are eliminated. Thus, the invention includes novel methods of maintaining the heating means and the strip passing through particular zones of the furnace at desired constant temperatures.

It is a further object of the invention to provide novel methods of controlling the hardness and ductility of the annealed strip, by controlling and varying the temperature in the soaking zone and the cooling rate.

A further object of the invention is to provide improved methods of and apparatus for cleaning the palm oil, employed in the cold rolling operation, from the surfaces of the strip steel. Another object is to eliminate the use of expensive apparatus and costly chemicals in the cleaning of palm oil from strip steel, thereby entirely eliminating the cost of preliminarily cleaning the steel, prior to annealing, which heretofore has always been necessary. For instance, in batch annealing processes, the cost of cleaning the palm oil from the strip amounts to about \$1.10 per ton, and the oil and cleaning chemicals are entirely wasted.

35 A further object of the invention is to convert a cleaning operation from a liability into an asset, by reducing the electric current consumption required to raise the steel to the annealing temperature. To this end, the invention contemplates burning the palm oil from the strip steel in the heating chamber and using the heat generated during the combustion of the palm oil to assist, at least in part, in raising the temperature of the strip to the annealing temperature.

40 45 A further object of the invention is to burn the palm oil from the strip steel, to clean the latter, without destroying the non-oxidizing character of the atmosphere in the annealing and cooling chambers.

45 50 A further object is to improve the heat absorptive characteristics of the strip steel by introducing it into the heating chamber with its surfaces in a dull, non-reflective condition, because of the presence of a film of palm oil thereon.

55 It has been discovered that, because of the dull,

oiled condition of the surface of the strip, it has approximately two and one-half times the heat absorptive qualities of a bright, dry reflective strip, previously cleaned in an alkaline solution.

A further object of the invention is to so regulate the burning of the palm oil on the surfaces of the strip that a clean, complete and efficient combustion takes place, leaving substantially no carbon deposit in the heating chamber, but without introducing an excess of oxygen, which would adversely affect the non-oxidizing character of the atmosphere.

Other objects and advantages of the invention will be apparent from a consideration of the following description of certain specific embodiments of the invention shown in the accompanying drawings.

In the drawings:

Figure 1 is a side elevation of a preferred form of annealing apparatus with certain parts removed for the sake of clarity, and with certain parts shown somewhat diagrammatically;

Figure 2 is a vertical section view of the heating section of the annealing furnace of Figure 1, on a somewhat enlarged scale, with certain parts removed and other parts broken away;

Figure 3 is a transverse sectional view taken on line 3—3 of Figure 2;

Figure 4 is a top plan view of the apparatus in Figure 1 with certain parts removed;

Figure 5 is an enlarged fragmentary vertical section through one of the heating chambers showing a preferred arrangement of heating elements;

Figure 6 is a sectional detail, showing a preferred terminal arrangement;

Figure 7 is a vertical sectional view of one of the caps or hoods for closing the upper end of one of the heating chambers;

Figure 8 is a horizontal sectional view showing the furnace floor in plan;

Figure 9 is a side view, on an enlarged scale, partly in section and partly in elevation, showing the lower end of the furnace structure and the strip guiding means;

Figure 10 is a fragmentary vertical section taken on line 10—10 of Figure 9;

Figure 11 is a plan view of the furnace casing, with the brickwork, guiding rolls and closure hoods removed;

Figures 12 and 13 are sectional details taken on corresponding section lines on Figure 11;

Figure 14 is a plan view of a channel-forming frame member or collar adapted to be mounted at the upper ends of the side walls of the furnace casing;

Figure 15 is an end elevation of the member shown in Figure 14, while Figures 16 and 17 are sections on corresponding section lines on Figures 14 and 15;

Figure 18 is a plan view of the hood or cap shown in Figure 7, while Figures 19 and 20 are an elevation and a vertical section thereof, the latter being taken on line 20—20 of Figure 19;

Figure 21 is a vertical sectional view of a gas-tight roll seal through which the strip passes to the annealing apparatus, and

Figures 22 and 23 are side and front elevational views of the apparatus of Figure 21.

As explained in detail in the above identified applications, the strip steel 10 is drawn from any suitable source of supply, such as one of a plurality of coils of strip, through a looper 70, a heating furnace 119 and a plurality of cooling chutes, in which the strip is reduced to a non-oxidizing

temperature before it is exposed to the atmosphere. The strip passes beneath a guide roll 90 and then through a looper, as explained in the above identified applications and to a reeling device. Master pinch rolls may be interposed between the guide roll 90 and the looper on the discharge side, to draw the strip through the apparatus, as described in those applications.

On its way to the furnace, the strip passes 10 to the first one of a plurality of lower rolls 11 of the looper 70, the rolls being journaled on a fixed lower frame 72. A plurality of upper rolls 73 are journaled on a vertically movable frame 74, supported by cables 75 and an appropriate counterweight, not shown. The strip passes over the several rolls in a serpentine path, to provide a reserve supply of strip between the main supply, constituted by a plurality of coils, and the entrance guide roll 76 of the annealing furnace, to 20 permit the strip, behind the looper 70 to be stopped while the leading end of a new coil of strip is welded to the trailing end of an exhausted coil, while permitting a continuous delivery of strip from the looper to the annealing furnace. 25 It will be understood that, while the delivery of strip to the looper is arrested, to permit the making of such a weld, the upper frame 74 of the looper is drawn downwardly against the action of its counterweight, to permit the continuous delivery of strip to the furnace. As soon as the welding has been completed, the strip is delivered to the looper at a speed above normal, to replenish the supply in the looper, while continuing the delivery of the strip to the furnace.

35 The furnace proper is supported by a suitable framework comprising upright structural members 115, a lower platform 116, and upper, horizontal frame members 117. The frame may be braced by suitable tie rods 118, or the like. The platform 116 supports the furnace casing 119 made up of a plurality of relatively heavy sheet metal sections continuously welded along their meeting edges and reinforced by suitable angle bars and the like to provide a strong, substantially gas-tight casing structure. Referring to Figures 2, 3, 5, 8 and 9, within the casing 119 and supported by the platform 116, there is a refractory brickwork floor 120, and similar side walls 121, 122, front and back end walls 123 and vertically extending partitions 124, 125 and 126, providing four vertical heating chambers 127, 128, 129 and 130. The floor 120 is provided with a plurality of relatively narrow openings 127a—130a, registering, respectively, with the vertical furnace chambers. At their upper ends, the chambers terminate in restricted throats 127b—130b, respectively, which communicate with roll chambers 131, 132, lined by continuations of the side and end walls and the vertical partition 125.

60 The space between the brickwork walls 121, 122 and 123 and the metal furnace casing 119, is packed with suitable heat insulating material, such as rock-wool, asbestos, or the like.

At the lower ends of the vertical chambers 127—130, access doors 133 having suitably refractory lining 134 are supported for swinging movement to and from closed position by hinge bars 135 (see Figs. 1 and 8). Hence, the floor of the heating chambers may be inspected and cleaned from time to time.

At its upper end, the furnace casing is offset inwardly at 136 to provide two independent casing extensions defining the two roll-receiving chambers 131 and 132. The casing extensions terminate at their upper ends in two series of

flat, horizontally disposed plates 137, providing two rectangular bases (Fig. 17) for rectangular, channel-forming collars 138, one of which is shown in detail on an enlarged scale in Figures 16-19. As shown in Figure 16, each collar comprises an inner angle member 138a, and a vertical, outer plate 138b, continuously welded thereto and braced by triangular pieces 138c, thereby providing a marginal channel 138d which operates with a hood, described below, to provide a substantially gas-tight seal for each roll chamber.

As shown in Figures 11 and 12, the upper casing 135 and the horizontal base 137 for the collar 138 are recessed at 139 to provide spaces for the reception of water-cooled roll shafts herein-after described. Likewise, the collar 138 (Fig. 15) has an upwardly projecting recess 139', formed by a vertical plate 138e and a semi-cylindrical plate 138f, providing a rounded hump in the channel 138d, directly above the recess 139, when the parts are assembled.

The roll chambers 131, 132 are closed by hoods or caps 140, shown more particularly in Figures 7, 18, 19 and 20. Each hood comprises side and end walls 141, a curved top wall 142, suitably reinforced by angle straps 143 carrying lifting eyes 144, and a refractory brickwork lining 145 for the top and sides. The sides and end walls of each hood carry outwardly and downwardly projecting flanges continuously welded together and to the hood and providing a sealing skirt 146, having a free edge adapted to be received in the channel 138d of the collar 138, as shown in assembled relation in Figures 2 and 3. The end walls of the hoods, at opposite points, are recessed upwardly at 147 to provide a space aligned with the recesses 139, 139', to accommodate the water-cooled roll shafts previously mentioned. A semi-cylindrical plate 147a (Fig. 20) defines the recess and is positioned to embrace the shaft.

Rolls 150, 151 (Figs. 1, 2, and 4) are fixed to hollow shafts 150', 151', journalled in outboard bearings 152, 153 carried by the upper, horizontal frame members 117. The spaces between the shafts and the arcuate recesses 139, 139' and 147 of the roll housing structures are closed by packing glands 152', 153' (Fig. 4), bolted to the exterior face of the casing wall extensions 135 and the collars 138, bolt holes 135a being provided for that purpose (Figs. 14 and 15).

As stated above, the shafts 150', 151' are hollow for the circulation of cooling water through suitable connections at their ends, not shown. As the description of the present invention progresses, it will be apparent that many parts of the apparatus are water-cooled, but the cooling water circulating pipes have been omitted from the drawings, since they would only tend to obscure other parts.

Below the horizontal platform 116, there is a roll casing, representing generally at 155 in Figures 1 and 9. The casing comprises a floor member 155a, supported upon transversely disposed I-beams 156 and spaced, longitudinal girders 156a. Side walls 155b, and walls 155c and a ceiling 155d, provided with suitable openings 155e and a refractory, brickwork lining 157 are supported from the floor 155a. An access door 158, provided with a suitable refractory lining, is mounted for swinging movement in a manner similar to the door shown in Figure 8, whereby the casing may be inspected and cleaned.

The spaces between the casing walls and the brickwork lining 157 is filled with insulating ma-

terial 157a. The front end wall 155c is made up of a plate bolted to the reinforced margins of the casing surrounding an opening at that end. The plate may be removed and the insulation at that end broken down, if it is desired to remove the large roll from the interior of the casing for replacement or repair.

Both end walls of the casing 155 are apertured and provided with stuffing boxes 159 (Fig. 10), through which the hollow, water-cooled shaft 160 of the lower roll 161 projects, the shaft being journalled in outboard bearings 162 carried by suitable supporting brackets 163 mounted on the I-beams 156. Cooling water from a suitable header is conducted by suitable pipes through connections, not shown, to the hollow shaft, to maintain the same in reasonably cool condition.

Projecting through a stuffing box 164 secured to the end casing plate 155c, is a shaft 165, supported at its opposite end in an appropriate bearing in the opposite end wall, and carrying a scraper blade 166, which projects downwardly into contact with the periphery of the roll 161, to scrape any scale or dirt therefrom, so that a clean roll surface is always presented to the incoming strip of sheet metal. On its outer end, the shaft 165 carries an operating handle 167, whereby the position of the blade 166 and the tension with which it is urged downwardly onto the surface of the roll may be accurately determined. The blade is preferably a resilient, special alloy plate, substantially  $\frac{1}{8}$  of an inch in thickness, known in the trade as "resistal #7."

Beneath the roll casing 155 there are a pair of rolls 168 journalled on appropriate bearings adjacent the opposite ends of the spaced longitudinal girders 156a, whereby, upon occasion, the strip may be led over the roll 168 and under the rolls 168, to by-pass the annealing furnace entirely.

Disposed beneath the platform 116 and in substantial alignment with the final heating chamber 130, there is a second roll housing 170, having rolls therein adapted to guide the strip from the final heating chamber to the first cooling chamber. As shown in Figure 9, the housing 170 has an upper section 171 communicating through a water-cooled chute section 172 with the opening in the platform 116 which is aligned with the slit 130a in the furnace floor 120. A roll 173, disposed in the upper section 171, is fixed to a hollow, water-cooled shaft journalled for rotation in outboard bearings 174 carried by brackets secured in vertical channels 174' extending between supporting I-beams 182 and the furnace platform. Appropriate stuffing boxes surround the roll shaft to prevent the escape of gas. The sides of the casing are provided with suitable water-jackets 175, 175a, the latter of which is extended horizontally at 175b over the top wall of the casing proper. The strip is guided under the roll 173 and thence about lower rolls 176, 177, similarly journalled in bearings 178, 179. The bearings 178, like the bearings 174, are supported by the vertical channel 174', while the bearings 179 are carried by brackets 177. A dirt catching trough 173' extends lengthwise of the casing below the roll 173 and above the roll 176, to prevent the entrance of dirt or scale between the strip and the periphery of the latter roll. The side and end walls of the casing likewise are water-jacketed, as indicated at 180, 181, to maintain the rolls in reasonably cool relation and to extract heat from the strip passing through the casing. The casing

170 is supported by suitable I-beams 182 or the like.

The cooling section of the apparatus comprises a vertical frame including upright structural members 115a, a pair of upper horizontal I-beams 117a, transverse members 117b, and intermediate transverse members 117c. The upper frame members 117b and 117c support two pairs of casing assemblies, providing four similar roll housings 195, 195a, 195b and 195c, each of which has communication with a pair of vertical chutes. The first housing 195 preferably is provided with outboard bearings 196 (Fig. 4) for a hollow, water-cooled shaft 196', carrying the roll in that housing. The shafts for the rolls in the other roll housings may have bearings 197 associated with the end walls of the housings, since they need not be water-cooled. Each pair of housings 195, 195a and 195b, 195c is mounted upon an individual base 198, supported on the transverse frame members 117b and 117c.

Certain of the cooling chutes are supported by roll housings 200, 200a, 200b (Fig. 1), each of which is made up of two sections similar to the casing section 170a of the roll housing 170. The first casing 200 is provided with outboard bearings 201 for the hollow water-cooled roll shaft, while the other two may have bearings 202 carried directly by the casing end walls.

The strip passes under the roll 177 and is drawn upwardly through a casing section 170a, which, at one side, is bolted, with a suitable gasket interposed, to the casing 170 and at its upper end 170b is provided with a flange which may be similarly bolted to the lower end of a first water-cooled, cooling chute section 185 (Fig. 1).

The strip passes from the cooling chute section 185 over a guide roll in an upper casing 195 to a second cooling chute made up of sections 203 arranged end to end, and from this section through a casing 200 at the lower end thereof to another cooling chute made up of similar sections 203, arranged end to end. The sections 203 may be cooled by the exposure to external atmosphere alone, or may have water jackets associated therewith. At the upper end of the last mentioned section, the strip passes through a casing 195a and then successively through cooling chutes 210, 211, and 213. It will be noted that these sections are connected together by casings 200a, 195b, 200b and that a casing 195c is connected to a final chute 235.

The chutes 210, 211, 212 and 213 are made up of sections having devices associated therewith for cooling the atmosphere in the chutes and for positively circulating the same over the surfaces of the strip passing therethrough. Preferably, these devices take the form of cooling units 219, carried by the chute sections and constructed in accordance with the specific disclosure of Figures 41 and 42 of our patent and application identified above. Since the cooling units are not claimed in this application, their details of construction will not be described herein.

If desired, one or another of the cooling and gas circulating assemblies may be removed from its associated chute and a simple flat plate, or a water-jacketed plate, substituted, depending upon the rate of cooling desired. In the alternative, one or another of the fans may be disconnected and rendered inoperative, to decrease the cooling effect of that section. Moreover, the speed of rotation of the fans and the volume of flow of cooling water through the cooling coils

may be independently varied at will, to control the effective cooling of the various sections.

A preferred drive for the fan units is shown in Figure 1. Certain of the transverse channel members 207, 207a, etc., carry upwardly projecting brackets 400 having bearings 401 at their upper ends, in which one or another of the shafts 402 are journaled. The transverse channel members also support motor brackets 405 carrying motors 406, connected to the shafts 402.

As indicated in Figure 1, each shaft 402 drives a bank of eight fan units, by means of sprockets 407 and upwardly and downwardly extending sprocket chains 408, 409, trained about similar sprockets 410, 411 on the fan shafts. The upper chains 408 incline upwardly and rearwardly from the axis of the shaft 402 to the axis of the several fans in the upper fan casings, while the lower sprockets 409 incline downwardly and rearwardly toward the sprockets associated with the lower fans.

Thus, the twenty-four fan units in the arrangement disclosed in Figure 1 are arranged in three banks of eight units each, and three driving assemblies and motors serve to drive them all.

The final cooling chute 235, which is disposed behind the vertical I-beam 115a in Figure 1, comprises a plurality of sections similar to the sections 203 which are cooled by room air alone.

30 A roll seal assembly, generally similar to the one shown in Figures 21-23, but omitting the means for introducing controlled amounts of air, as hereinafter explained, may be suspended from the lowermost chute section 235 or from the 35 transverse supporting channels 241 (Figure 1). Since this assembly is substantially identical to the assembly 245 carried by a downwardly projecting water-jacketed throat 246 associated with the first heating section 127 (Figure 9) of 40 the annealing furnace, only the latter roll seal assembly will be described, reference being had particularly to Figures 21-23.

Each seal assembly includes an upper housing member which is preferably a unitary casting including side walls 247, 248, upper attaching flanges 249 and end walls 250. The end walls 250 terminate in outwardly projecting wings 251, to which roll supporting brackets 252, 253 may be attached, the former being a stationary roll bracket, secured by four bolts 252', and the latter being a movable bracket pivoted for limited swinging movement about the axis of an attaching bolt 254. Rolls 255, 256, fixed upon shafts 257, 258, are journaled in bearings 259, 260 carried, respectively, by the fixed and pivoted roll supporting brackets. The brackets are provided with downwardly projecting arms 261 and 262, connected together by an adjustable link 263 and a tension spring 264, whereby the movable roll supporting brackets and the roll 256 are urged constantly toward the stationary brackets and the fixed roll 255.

The downwardly projecting side flanges 247, 248 of the main housing carry elongated sealing bars 266 of hard packed felt, or the like, urged downwardly into contact with the roll peripheries by compression springs 267, surrounding bolts 268 depending from the flanges 249 and interposed between nuts 269 and shoes 270. The bars 266 are pressed inwardly into firm sealing contact with the flange 247, 248 by presser strips 271 and compression 272, surrounding bolts 273 and urged inwardly by nuts 274. This construction provides a substantially gas-tight seal between the sides of the strip and the rolls and be-

tween the rolls and the side walls of the main housing.

A seal is effected between the end walls 250 of the housing and the rolls 255, 256 by hard, pressed felt, end dam members 275, urged inwardly toward the outer face of the end walls by presser plates 276. The end dams 275 and the plates 276 are provided with arcuate cut-out corners 277, 278, in peripheral engagement with reduced end portions 279 of the rolls 255, 256. These members are supported by bolts 280 and are urged inwardly against the end faces 283 of the rolls 255, 256 by springs 281 and nuts 282.

Hence, a substantially gas-tight seal is provided. The only space through which gas may pass is the small space between the rolls 255, 256 at the ends thereof, between the strip passing through the rolls and the end dam members.

As stated above, one of the principal objects of the invention of the present application is to burn off the palm oil applied to the surfaces of the strip steel during the cold rolling operation, to clean the strip and to assist in maintaining the desired high temperature in the heating chamber. This burning of the palm oil is made possible by the introduction of sufficient air to support combustion of the highly heated and volatilized oil. If air is not so introduced, the strip will be cleaned by volatilization of the oil, but the oil will be broken down into hydrocarbon gases and amorphous carbon, which collects in the first leg of the furnace and which must be removed from time to time. Although this removal of the carbon may be effected quite simply, by introducing relatively large volumes of air into the furnace and maintaining the electric heating elements energized, thereby burning out the carbon deposit, the delivery of strip to the furnace must be discontinued while the carbon cleaning operation is going on, thereby causing an interruption in the production of annealed strip steel.

We have discovered that, by continuously introducing a controlled amount of air, the palm oil may be volatilized and cleanly burned as the strip steel is continuously delivered to the apparatus, thereby avoiding the necessity for shutdowns to clean the furnace. Moreover, if the air so introduced is accurately controlled, the non-oxidizing character of the atmosphere in the furnace is not adversely affected, and the heat from the burning oil is utilized to assist in maintaining the desired temperature in the furnace, thereby decreasing the consumption of electric current.

The air may be introduced directly above the roll seal assembly at the entrance end of the apparatus, for instance, by a pipe extending into the water cooled throat 246 (Figure 9) or by a pipe or hose 290 connected to a nipple 291 of accurately predetermined internal diameter in the end wall 250 (Figs. 22 and 23) of the upper housing member for the roll seal. With an apparatus of the size and capacity contemplated and described in this application, a one-quarter inch orifice supplied with air under eight pound pressure per square inch, delivers the right amount of air to burn off the oil on the strip. The conduit 290 may lead from a pressure regulator 292 and a storage tank 293, supplied with air under pressure by a compressor 294. Air at eight pounds pressure forced through a one-quarter inch orifice in this manner will be delivered to the heating chamber at the rate of nineteen cubic feet per minute. Strip steel of the gauge employed in the manufacture of crown closures and can ends, between 29" and 31" in

width, carries between  $\frac{1}{2}$  and  $\frac{3}{4}$  lbs. of palm oil per ton. If the apparatus is operating at about ten tons of steel per hour (three hundred and thirty lbs. per minute) this amount of air will efficiently support combustion of the oil.

An analysis of the atmosphere in the heating chamber is as follows: CO—16.1%; CO<sub>2</sub>—3.8%; O—0.0%. In the cooling chamber, the atmosphere has the following analysis: CO—12.9%; CO<sub>2</sub>—5.1%; O—0.0%.

The temperature increase in the first ten zones of the annealing furnace, resulting from the burning of the palm oil by the introduction of air is indicated in the following table:

|    | Zone No. | Air Off | Air On | Temp. Increase |
|----|----------|---------|--------|----------------|
| 20 | 1        | 1,385   | 1,465  | +70            |
|    | 2        | 1,430   | 1,500  | +80            |
|    | 3        | 1,430   | 1,490  | +60            |
|    | 4        | 1,455   | 1,515  | +60            |
|    | 5        | 1,535   | 1,600  | +65            |
|    | 6        | 1,545   | 1,610  | +65            |
|    | 7        | 1,540   | 1,600  | +60            |
|    | 8        | 1,470   | 1,530  | +60            |
|    | 9        | 1,590   | 1,645  | +55            |
|    | 10       | 1,660   | 1,725  | +65            |

Except for the means for introducing a controlled amount of air, the only difference between the two gas-tight roll seals at the entrance end of the annealing furnace and at the discharge end of the last cooling chute is that the rolls 255, 256 of the entrance assembly are steel, while at the outlet, it is preferred to use tightly packed cloth disc rolls. Rolls of the latter type consist of a plurality of circular, radially disposed cloth discs threaded on an axial shaft and subjected to axial compacting pressure. Since such rolls are known in the art, they are not shown specifically herein.

In some cases, it has been found desirable to positively drive the rolls 255, 256 at the entrance end of the apparatus, since the strip at that time is coated with palm oil and is quite slippery. To this end, the roll shafts may be provided with intermeshing pinions, to cause the rolls to move in unison, and one of the shafts may carry a pulley 257', driven by a belt 257a, trained about a pulley 257b carried by the first guide roll 76 (Fig. 9).

All of the various individual parts of the casing sections, chute sections, roll housing sections and the like are preferably welded together with continuous welds to provide gas-tight seams. The individual sections in turn are preferably bolted together with gaskets interposed between the joints, so that the apparatus, as a whole, is substantially gas-tight. When it is necessary to remove one part from another, or otherwise to disassemble the apparatus, the bolts may be readily removed and the sections taken down.

As a result of this construction, leakage of gas from the interior of the furnace and from the cooling chutes is reduced to a minimum. The gas-tight roll seals likewise prevent substantial dissipation of gas, while permitting a rapid delivery of the strip into and out of the sealed chambers. A suitable non-oxidizing, hydrocarbon gaseous atmosphere is maintained by continuously delivering a supply of such gas to the interior of the furnace, preferably through four pipe connections, one leading to each heating chamber adjacent the lower end thereof, on the opposite face of the furnace from that shown in Figure 1, as indicated at 127c, 128c, 129c, and 130c in Figure

2. It has been found satisfactory to maintain the gas in the annealing apparatus at a pressure between .2 and .5 inch of water above outside atmospheric pressure.

The atmosphere of non-oxidizing gas, maintained in the heating and cooling chambers, may be produced by burning clean fuel gas with an insufficient supply of air in a combustion chamber independent of, but in controlled communication with, the chambers. It is important that the gas be thoroughly dried before it is piped to the heating and cooling chambers. A suitable composition of the gas, as pointed out in the application and patent identified above, comprises:  $\text{CO}_2$ —5-6%;  $\text{CO}$ —10-12%;  $\text{H}_2$ —10-13%;  $\text{N}_2$ —balance. Obviously, the composition may be varied as desired between wide limits, so long as a non-oxidizing atmosphere is maintained, to prevent oxidation of the surfaces of the highly heated strip.

Referring to Figures 3 and 5, the strip is heated during its passage through the chambers by radiations from a plurality of banks of radiant electric heating elements 300, 300a and also by the highly heated atmosphere in the chambers. As shown in Figure 5, the heating elements are preferably arranged in banks comprising four rows of loops or festoons, each constituting a series continuation of the next. One row of festoons 301 is supported by hanger lugs 302 comprising integral projections associated with insulator blocks, built into the brickwork of the furnace. Each series of blocks, in the arrangement shown, includes seven triple hanger blocks, each having three lugs thereon, and one single hanger block. An important feature of the heating elements is that the festoons gradually and progressively increase in length from opposite ends toward the middle. For instance, the middle loops may be substantially 6.6", while the end ones are 3.8", measured from the top of the hanger lugs to the bottoms of the festoons. Each series may include twenty or twenty-one downwardly projecting loops and the loops may be formed from the .128" by 1" NiCr ribbon.

The variation in the lengths of the loops prevents overheating of the edges of the steel strip being annealed and provides a substantially uniform temperature gradient entirely across the strip. Preferably, the longer loops 305 at the center of each series are positively maintained out of contact with each other by guiding projections or lugs carried by special insulating guide blocks 304, mounted in the furnace wall, below the hanger blocks.

The heating elements are arranged in banks of four rows of festoons, connected in series at their ends by continuations 306, 307, and 308, the elements and supporting and guiding means of each row being of the same construction. The ends 310 of the heating elements project rearwardly through the furnace brickwork and insulating material, where they are doubled back upon themselves, as at 311 (Figure 6) and welded together and welded to the bifurcated end 312 of a binding post 313, the latter being carried by an insulating plate 314 secured to the furnace casing by bolts 315 or the like, in gas-tight relation with an appropriate gasket interposed between the plate and a reinforcing strip 316 welded to the casing around the opening for the binding post. The binding post 313, which is preferably of Monel metal, has a Monel collar 313' welded thereto, carrying a plurality of pins 317 projecting into sockets formed in the insulating plate

314, to prevent twisting of the post and the heating element when the post is clamped to the insulating plate by a nut 318, or when a bus bar or the like is bolted to the outer end of the post by nuts 319.

It will be understood that similar banks 300, of heating elements are mounted on both side walls of each heating chamber on opposite sides of the strip steel being drawn therethrough. Each bank, similar to that shown in Figure 5, and comprising four rows of loops, will be connected in series, by external connections to the corresponding bank on the opposite side of the strip steel. Each pair of banks thus connected constitutes a single heating zone. As pointed out in the application and patent identified above, the elements constituting each zone are connected in parallel to a source of current, and individual control means are provided for each zone. A pyrometer tube 325 is provided for each zone, projecting through the furnace end wall between the middle rows of elements, as shown in Figure 5 and as indicated by the dotted circles 325 in Figure 2.

Each bank of heating elements in the heating chambers 127, 128 and 129 has a 30 kilowatt rating, so that, in each chamber, eight 60 kilowatt heating zones are provided. In the final chamber 130, the elements are constructed of  $\frac{3}{4}$  inch ribbon, with the result that each bank has a 20 kilowatt rating, thereby providing a plurality of 40 kilowatt zones. Preferably, in the final heating chamber there are only four such zones.

By connecting the elements of different zones in various ways, as for instance, by connecting all of the elements of two or more zones in series with each other, or by disconnecting some of the elements entirely by the control devices, appropriate heating conditions for a wide variety of gauges and widths of strip can be effected.

We claim:

1. An apparatus for continuously cleaning the oil from the surfaces of cold rolled strip steel and for continuously annealing the strip, comprising heating and cooling chambers in communication with each other, substantially gas-tight seals at the entrance and discharge ends of the chambers, means for drawing strip through the seals and the chambers, means for maintaining a non-oxidizing atmosphere in the chambers, and means for burning the oil from the strip in the heating chamber, the last-mentioned means comprising an orifice of predetermined size communicating with the interior of the heating chamber, an air line leading to said orifice and means for delivering air to the line at a predetermined constant pressure, whereby air is delivered to the heating chamber at a controlled rate to support combustion of the oil and to assist in maintaining the temperature in the heating chamber at the desired elevation.

2. An apparatus for continuously annealing strip steel and for cleaning the cold rolling lubricant from the surfaces thereof, comprising a plurality of parallel, interiorly communicating, vertically disposed heating and cooling chambers, means for guiding the strip into, through and from the chambers, means for introducing non-oxidizing gases to the chambers to produce a non-oxidizing atmosphere therein, sealing means at the entrance and exit ends of the chambers for preventing the admission of atmospheric air as the strip enters and leaves, heating means in heating chambers, cooling means in cooling chambers, an orifice of accurately predetermined

size opening into the first chamber above the seal, and means for delivering air to and through the orifice under predetermined pressure, whereby sufficient air is introduced to support combustion of the lubricant in the first heating chamber, without destroying the non-oxidizing character of the atmosphere.

3. An apparatus for continuously annealing cold rolled strip steel and for cleaning the lubricant from its surfaces, comprising elongated intercommunicating heating and cooling chambers through which the strip is drawn, a gas-tight seal at the exit end of the cooling chamber, and means for preventing the inadvertent admission of air at the entrance end of the heating chamber and for continuously delivering thereto, air at an accurately controlled rate, the last mentioned means comprising a casing communicating with the heating chamber and having side and end walls defining a passage through which the strip is drawn, a roll aligned with and journalled for rotation on a fixed axis below one side wall, a second roll aligned with and journalled for rotation below the other side wall and mounted for limited movement toward and from the first roll, means for urging the second roll toward the first, sealing means between each side wall and the associated roll periphery and between the casing end walls and the rolls, whereby air is prevented from entering the chamber with the strip passing between the rolls, an orifice of predetermined size through one of the walls of said casing, and means for delivering air under accurately controlled predetermined pressure through the orifice and into the casing above the rolls to support combustion of the lubricant on the strip.

4. For use with a continuous annealing apparatus of the type comprising heating and cooling chambers through which the strip steel is drawn, means for preventing the inadvertent admission of air with the strip at the entrance end of the chamber and for delivering air at an accurately controlled rate to the chamber to support combustion of the cold rolling lubricant on the strip, said means comprising a casing communicating with the chamber, a pair of rolls journalled below the casing, sealing strips carried by the casing, spring means for urging the strips into contact with the roll periphery, end dam members carried by the casing, spring means for urging said members into contact with the end faces of the rolls, whereby air is prevented from entering the casing as the strip passes between the rolls, an orifice extending through the casing, and means for delivering air at an accurately controlled rate through the orifice.

5. A substantially gas-tight roll seal for the entrance or discharge ends of a strip annealing apparatus or the like, comprising a casing through which the strip passes, a pair of fixed brackets projecting downwardly from opposite ends of the casing, a pair of movable brackets projecting downwardly from the opposite ends of the casing, fixed and movable rolls journalled respectively in the fixed and movable brackets, resilient means urging the movable brackets and roll toward the fixed brackets and roll, sealing strips carried by the side walls of the casing with their lower faces in contact with the adjacent roll peripheries, end dam members carried by the end walls of the casing with their lower portions in contact with the end faces of the rolls, and a plurality of springs for maintaining said sealing

strips and said end dam members in such contact with the rolls.

6. A substantially gas-tight roll seal for the entrance or discharge end of a strip annealing apparatus or the like, comprising a casing through which the strip passes, a pair of fixed brackets projecting downwardly from opposite ends of the casing, a pair of pivoted brackets projecting downwardly from the opposite ends of the casing, fixed and movable rolls journalled respectively in the fixed and pivoted brackets, resilient means urging the movable roll toward the fixed roll, sealing strips along the lower margins of the casing side walls, means for urging the strips into contact with the side walls, means for resiliently urging the strips into contact with the roll peripheries, sealing plates adjacent the lower margins of the casing end walls, and means resiliently urging the plates into contact with said end walls and with the end faces of the rolls.

7. A substantially gas-tight roll seal for use with the entrance or discharge end of a continuous strip annealing apparatus or the like, comprising a casing having side and end walls defining a passage through which the strip is drawn, a laterally projecting flange at the upper end of the casing for attaching the same to the apparatus, a fixed roll aligned with and journalled for rotation below one side wall, a second roll aligned with and journalled for rotation below the other side wall and mounted for limited movement toward and from the first roll, means for urging the second roll toward the first, a sealing strip between each side wall and the associated roll periphery, sealing plate means for closing the spaces between the casing end walls and the rolls, and means for urging the sealing strips and the sealing plate means into contact with the rolls.

8. A substantially gas-tight seal for the entrance or discharge end of a strip annealing apparatus or the like comprising a casing through which the strip passes, having vertically disposed, horizontally elongated side walls and relatively narrow, vertically disposed end walls, a pair of rolls journalled below the side walls on horizontal axes parallel thereto, elongated sealing strips carried by the side walls of the casing, spring means for urging the strips downwardly into contact with the roll peripheries, means projecting from each end wall of the casing, an end dam member carried by each of the last mentioned means having a sealing face in contact with the adjacent casing and wall and with the adjacent end faces of the rolls, and compression spring means carried by each of the last mentioned means urging the end dam members into such contact.

9. A substantially gas-tight seal for the entrance or discharge end for a strip annealing apparatus or the like, comprising a casing through which the strip passes, having vertically disposed, horizontally elongated side walls and relatively narrow, vertically disposed end walls, a pair of rolls journalled below the side walls on horizontal axes parallel thereto, elongated sealing strips carried by the side walls of the casing, spring means for urging the strips into sealing contact with said walls, spring means for urging the strips downwardly into sealing contact with the roll peripheries, an end dam member carried by each end wall of the casing, and spring means supported by the casing end walls for urging the end dam members axially and in-

15

wardly into sealing contact with the end walls and with the end faces of the rolls.

WILLIAM B. COOPER.  
EDWARD J. SEABOLD.

## REFERENCES CITED

The following references are of record in the file of this patent:

## UNITED STATES PATENTS

| Number    | Name      | Date          | Number     | Country       | Date         |
|-----------|-----------|---------------|------------|---------------|--------------|
| 814,124   | Fish      | Mar. 6, 1906  | 10 114,754 | Germany       | Nov. 1, 1900 |
| 1,546,532 | Baily     | July 21, 1925 | 10 417,657 | Great Britain | Oct. 4, 1934 |
| 1,696,900 | Baily     | Jan. 1, 1929  |            |               |              |
| 1,713,485 | Alexander | May 14, 1929  | 15         |               |              |
| 1,719,793 | Alexander | July 2, 1929  |            |               |              |
| 1,732,917 | Summey    | Oct. 22, 1929 |            |               |              |

16

| Name     | Date          |
|----------|---------------|
| Harris   | July 13, 1937 |
| Keller   | Oct. 15, 1940 |
| Capstaff | July 14, 1942 |
| Cook     | May 18, 1943  |
| Renkin   | Jan. 9, 1945  |

## FOREIGN PATENTS

| Number  | Country       | Date         |
|---------|---------------|--------------|
| 114,754 | Germany       | Nov. 1, 1900 |
| 417,657 | Great Britain | Oct. 4, 1934 |

## OTHER REFERENCES

Industrial Furnaces, by W. Trinks, vol. II, published 1925 by John Wiley & Sons, Inc., New York, N. Y. pp. 217-218, paragraph entitled "Furnace atmosphere in electrically heated furnaces."